

April 23, 1968

J. R. ROBERTS

3,379,609

WATER-FELTED BUILDING PRODUCT INCLUDING  
NONFIBROUS CELLULOSE BINDER  
Filed Jan. 16, 1964



INVENTOR.

James R. Roberts  
BY  
Fordham, Newman,  
Schild & Williams  
attorneys

1

3,379,609

**WATER-FELTED BUILDING PRODUCT INCLUDING NONFIBROUS CELLULOSE BINDER**  
James R. Roberts, Palatine, Ill., assignor to United States Gypsum Company, a corporation of Delaware  
Filed Jan. 16, 1964, Ser. No. 338,057  
8 Claims. (Cl. 162—181)

**ABSTRACT OF THE DISCLOSURE**

A building product comprising expanded perlite, and a water-activated cellulose binder which is essentially nonfibrous in character.

This invention relates to the production of unified monolithic building products and more particularly to improved unified, lightweight building products in sheet form containing perlite and a cellulosic binder.

Expanded perlite is a well known commercial lightweight mineral aggregate, produced by the thermal expansion of the volcanic glass perlite. The product is cellular or vesicular in form, ordinarily having an essentially spherical shape. Generally the product produced by commercial operations contains a broad range of particle sizes.

Building products containing expanded perlite and fibrous materials such as paper pulp are also known. For example, prior art discloses insulating board products made from expanded perlite and newspaper pulp by accumulation on a cylinder machine from a slurry in a manner similar to paper manufacture. While these products have merit as insulating materials, it has been found that they lack sufficient structural integrity for certain purposes and do not have the necessary surface properties for use as finished wall or ceiling surfaces on residential or commercial construction. None of these products had any particular resistance to abrasion or compression.

Some attempts have also been made to improve the structural integrity of perlite-paper pulp products by the use of binders such as asphalt and other organic material such as starch, polymers and the like. While these expedients had some success in improving integrity of the product, they also changed the appearance and other properties of the product with respect to color, weight or fire resistance.

Accordingly it is an object of the present invention to provide an improved unified monolithic building product in sheet form which has characteristics of lightweight and superior strength.

A further object is the provision of a building product which has superior compression and abrasion resistance.

A still further object is the provision of a building product which has excellent structural integrity achieved without the use of synthetic organic fibers, asphalt or other synthetic binders.

Another object is the provision of a monolithic building product which has excellent fire resistance.

Another object is the provision of a monolithic building product in sheet form which has improved sound absorption and attenuation properties.

Another object is the provision of a unified building product in sheet form which has surfaces which are adapted for finishing.

Another object is the provision of a building product in sheet form which has superior thermal insulating properties.

The fulfillment of these and other objects of the present invention may be seen from the following specification and appended claims.

Accordingly in one broad form the present invention

2

comprises a unified lightweight monolithic building product in sheet form, said unified product comprising one part of a mechanically induced water activated cellulosic binder and from about 5/3 to 9 parts by weight (dry basis) of a thermally expanded perlite. Preferably the proportions of perlite range from 7/3 to 8.5 parts.

In another broad form the present invention comprises building products which contain a minor proportion of a ceramic clay, specifically up to about 2 parts clay per part of cellulosic binder, and in the most preferred instances from 1/3 to 2 parts of clay per part of cellulosic binder.

The foregoing compositions may also optionally contain boric acid as a fire retardant and small amounts of 15 a wax for water repellency. Waxes, such as microcrystalline wax, petroleum wax, paraffin waxes and the like, are suitable. The wax, when used, is usually in amounts up to about 2 percent by weight and preferably from 0.25 to 1 percent by weight. The boric acid is generally incorporated into the product in amounts up to 3 percent by weight, and preferably from 0.25 percent to 2 percent. 20 Alum may also be incorporated for superior processing in amounts of from about 1/2 to 1 1/2 percent. The minor additives, i.e. boric acid, wax and alum, are expressed as 25 percentages of the total product weight. All parts and percentages referred to herein, unless otherwise stated, should be understood to be on a dry weight basis.

Generally the products of the present invention are 30 lightweight, i.e. having densities in the broadest aspects of from about 4 to about 25 pounds per cubic foot, preferably from 8 to 20 pounds per cubic foot.

The proportions of the components of the products 35 of the present invention can be more particularly defined in terms of percent by weight. Broadly these products contain from 50 to 90 percent perlite, from 10 to 30 percent cellulosic binder and from zero to 20 percent clay. For example, those embodiments which consist essentially of cellulosic binder and perlite broadly contain from 70 to 90 percent perlite, from 10 to 30 percent 40 cellulosic binder. These products are eminently suitable for applications as insulating floor underlayment, ceiling or wall tile or insulating board. They are characterized by superior compressive strength and resistance to abrasion, sharp blows and abuse. These particular qualities of 45 a high perlite product make possible applications for a thermal insulating floor underlayment for surfacing with wood or plastic tiles that will stand up under the stress of floor traffic. This product may also be used in wall insulation and in tiles showing superior performance in the 50 area of insulation and reduction of sound transmission. This latter property is especially valuable in modern commercial buildings which feature suspended ceilings and non-loadbearing partition walls. Ordinarily in such construction the ceilings and walls are formed of tile or board. With the superior sound attenuation and deadening 55 properties available in these products the amount of sound transmission through the ceiling and walls into adjacent areas is substantially reduced, especially in those board products containing a high proportion of perlite.

The compositions of the present invention which contain clay in addition to perlite and cellulosic binder are especially useful in fire resisting applications. The clay used is of the high alumina and silica, ceramic variety and is characterized as nonswelling. Clays, such as kaolin, fire clay, brick clay and ball clay, are exemplary. The first resistant building product contains from about 50 to 80 percent perlite, from 10 to 30 percent cellulosic binder and from 10 to 20 percent ceramic clay. The clay is especially valuable in the production of fire rated tile. Thus, when subjected to fire, the clay containing tiles or 60 wallboard products sinter, rather than spall or undergo

gross delamination or support combustion, as in the case of other materials.

The products of the present invention may, as previously pointed out, also be used in the production of building materials for sound and thermal insulation wherein the surface is exposed to view.

Particular reference is also made to ceiling tile or board products of the present invention which may be painted, or if desired surfaced on one or both sides with paper sheets to form a laminated or sandwich construction. The products may also be used to prepare acoustical, drilled or perforated tile by conventional techniques.

The perlite which is used in the products of the present invention may be of a variety of mesh sizes. Generally mesh sizes of less than 8 mesh are suitable for structural insulating boards and underlayment. For those applications which require a smooth finish on the surface of the product, i.e. ceiling tile, it is preferred to use a finer perlite, preferably one in which at least 70 percent passes a 20 mesh screen, and which has no particles larger than 8 mesh (U.S. Standard Sieve Series).

The cellulosic binder, the manufacture of which is one aspect of this invention, is a highly hydrated gelatinous substance. The starting material may be any cellulosic material, preferably an unbleached waste kraft stock. It has been found that extended refining of the pulp results in a change of properties and the cellulose is converted thereby from a fibrous material to an essentially nonfibrous gelatinous substance. With this refining treatment it has been found that the properties of the cellulose change to such an extent that the material acts essentially as an adhesive without fiber interfelting action. The degree of hydration may be expressed in terms of Schopper-Riegler freeness. Preferably the products of the present invention are mechanically hydrated to a Schopper-Riegler freeness of less than about 100 ml. and preferably less than about 90 ml. The increasing hydration results in superior strength of the products when the cellulose material is used in the products of the present invention. The effect of the refining or Schopper-Riegler freeness is shown in the subjoined table.

TABLE 1.—FRENESS VALUES OF CELLULOSE BINDERS

| Pulp Sample                                        | Schopper-Riegler Freeness, ml. | Fiber Length, Index, num. <sup>1</sup> |
|----------------------------------------------------|--------------------------------|----------------------------------------|
| Unbleached waste kraft pulp stock <sup>2</sup> ... | 560                            | -----                                  |
| Series Refining:                                   |                                |                                        |
| After A                                            | 390                            | -----                                  |
| After B                                            | 170                            | -----                                  |
| After C                                            | 110                            | 0.061                                  |
| After D                                            | 80                             | 0.058                                  |

<sup>1</sup> See Forest Products Laboratory Report No. 884, reaffirmed 1956. Also, Schaefer and Carpenter, Paper Trade Jr. May 1930.

<sup>2</sup> After repulping: consistency 6-8+.

The series refining steps referred to in the above table are passes of the pulp through a Morden Stockmaker type pulp refiner equipped with lava tackle.

For a better understanding of this invention, reference is made to the accompanying drawing, illustrating in flow sheet form the sequence of steps involved in the process of the present invention. Referring to that drawing there is illustrated a paper source, preferably an unbleached waste kraft paper source, which discharges into a hydropulper of the Morden Slushmaker type, and water is added to form a kraft paper fiber furnish having a consistency of at least about 6 percent. The discharge from the hydropulper is passed to a stock tank and then through a series of pulp refiners (A, B, C, D), such as preferably of the Morden type equipped with lava tackle. The pulp from refiner A is discharged into a refiner B and thence to refiners C and D in cascade sequence with a total residence time of about 15 seconds. The final product has a Schopper-Riegler freeness of less than about 100. The cellulosic binder discharge from the refiner sequence is highly hydrated and essentially nonfibrous in character. The cellulosic binder is passed to a

stock tank for storage and supply. At intervals the cellulosic binder is passed to a mixing chest where perlite in the desired amount is added. Clay from source may also be added to the mix if desired in the particular embodiment. Water may be added from the source to adjust the consistency of the mix to from about 4 to about 8 percent although the consistency may also be adjusted in the furnish making stage. Other additives, such as boric acid, wax, and alum, as desired, may be added at this point. After mixing to form a uniform slurry, the contents of the mixing chest are discharged to the machine chest and thence onto the screen of the Fourdrinier machine. Other types of paper, board or sheet making machines, such as cylinder machines and the like may be employed, if desired. The slurry of cellulosic binder, perlite, and/or other additives is deposited or laid on the screen or wire in an initial thickness of from about 3/4 to 4 inches. The web thus formed is compacted in the press section by roller presses or the like to a thickness of from about 1/2 to 1 1/2 inches, and thence to a drier, preferably of the multiple deck variety. The dried product in sheet form is trimmed and cut to the desired size and passed to a storage or for further finishing, such as by painting, lamination of paper sheets on one or both surfaces, laminations of the sheet, perforations, or the like.

Insulation products were made by the process of the present invention containing varying amounts of perlite, cellulosic binder, clay and other additives. Each product was laminated with paper sheets on both surfaces to illustrate the results obtained with the laminated as compared with the unlaminated product. The following examples illustrate the composition and physical properties of the sheet products made in accordance with this invention.

## COMPOSITION OF SHEET

[All of the sheets were produced in a dry thickness ranging from 0.71 to 0.75 inch]

|                               | Perlite <sup>1</sup> | Cellulosic Binder <sup>2</sup> | Clay <sup>3</sup>     |
|-------------------------------|----------------------|--------------------------------|-----------------------|
| Example:                      |                      |                                |                       |
| 1                             | 90                   | 10                             | -----                 |
| 2                             | 85                   | 15                             | -----                 |
| 3                             | 62.5                 | 37.5                           | -----                 |
| 4                             | 83.3                 | 12.5                           | 4.2                   |
| 5                             | 70.8                 | 12.5                           | 16.7                  |
| 6                             | 62.5                 | 12.5                           | 25                    |
| UNLAMINATED SHEETS            |                      |                                |                       |
|                               | MOR <sup>4</sup>     | Density <sup>5</sup>           | Hardness <sup>6</sup> |
| Example:                      |                      |                                |                       |
| 1                             | 66                   | 12.3                           | 232                   |
| 2                             | 146                  | 13.5                           | 307                   |
| 3                             | 403                  | 13.8                           | 405                   |
| 4                             | 101                  | 12.5                           | 258                   |
| 5                             | 138                  | 13.1                           | 260                   |
| 6                             | 128                  | 13.1                           | 270                   |
| LAMINATED SHEETS <sup>7</sup> |                      |                                |                       |
|                               | MOR <sup>4</sup>     | Hardness <sup>6</sup>          |                       |
| Example:                      |                      |                                |                       |
| 1                             | 497                  | 295                            |                       |
| 2                             | 621                  | 335                            |                       |
| 3                             | 730                  | 380                            |                       |
| 4                             | 560                  | 300                            |                       |
| 5                             | 539                  | 255                            |                       |
| 6                             | 553                  | 275                            |                       |

<sup>1</sup> Parts by weight (dry basis). Screen analysis: +20 mesh 0%; +50 mesh 7.8%; +100 mesh 36.2%; +200 mesh 28.4%; -200 mesh 27.6%.

<sup>2</sup> Parts by weight (dry basis). Initial consistency, 6%. Schopper-Riegler Freeness less than 100.

<sup>3</sup> Parts by weight. Kentucky-Tennessee Clay Co. (CTS-1). Silica 57.0%; Alumina 27.9%; Loss on ignition 9.8%.

<sup>4</sup> Modulus of Rupture, Pounds per square inch.

<sup>5</sup> Pounds per cubic foot.

<sup>6</sup> Force in pounds required to force a 2 inch diameter steel ball 1/4 inch into the surface of the sheet.

<sup>7</sup> Laminated on both surfaces with manila faced chipboard sheet having a weight of 72 pounds per 1,000 square feet. Polyvinyl acetate adhesive (Du Pont Elvacet).

## Example 7

This example illustrates the commercial production of a lightweight insulation product of the present invention which has utility as a sound deadening board. The preparation follows the procedure described above. The following table shows the proportions of each component in the

final product in terms of percentage composition and weight.

|                            | Percent by weight | Pounds |
|----------------------------|-------------------|--------|
| Perlite                    | 62                | 4,960  |
| Cellulosic binder (solids) | 20                | 1,600  |
| Clay                       | 15                | 1,200  |
| Wax (solids)               | 1                 | 80     |
| Alum                       | 1                 | 80     |
| Boric Acid                 | 1                 | 80     |
| Total                      | 100               | 8,000  |

25,600 pounds of water and 1,600 pounds of unbleached waste kraft paper were introduced into a Morden Slush-maker and refined for 30 minutes. The resulting fiber furnish was passed into a stock tank and thence through a sequence of four Morden paper refiners (a throughput time of 60 minutes per ton).

The water activated cellulose binder from the last refiner had a Schopper-Riegler freeness of less than 100. The cellulosic binder dispersion at a consistency of about 6 percent was passed to a stock tank and then to a mixing chest for admixture with water (166,400 pounds), clay, perlite, boric acid, wax and alum in the amounts indicated. The perlite had a mesh size range of about -20 to +200 (70%). The clay was a ceramic type ball clay (Kentucky-Tennessee Clay Co., CTS-1) having the following analysis:

|                                | Percent |
|--------------------------------|---------|
| SiO <sub>2</sub>               | 57.0    |
| Al <sub>2</sub> O <sub>3</sub> | 27.9    |
| Ignition loss                  | 9.8     |

The wax was a microcrystalline wax—Mobil Oil Co. Mobilcere—RV emulsion.

The product from the mixing tank with a consistency of about 4 percent was passed to the Fourdrinier machine and formed into a sheet which, after pressing and drying, had a thickness of about  $\frac{3}{4}$  inch. The final product, when cut and trimmed, had a density of 14 pounds per cubic foot.

The products of the present invention are characterized by excellent fire resistance. For example, the products containing perlite, binder and clay have a class 1 rating by ASTM E84-61 (Underwriters Laboratories Standard 723). The products also have a Class A rating according to Federal Specification SS-A-00118c (Apr. 14, 1960).

As may be appreciated the cellulosic binder material and the water felted insulating and building products of the present invention are readily prepared in a variety of forms by the processes outlined above. The method described may also be modified with respect to the equipment used in manufacture, such substitution being conventional in this art.

While several particular embodiments of this invention are shown above, it will be understood, of course, that the invention is not to be limited thereto, since many modifications may be made, and it is contemplated, therefore, by the appended claims, to cover any such modifications as fall within the true spirit and scope of this invention.

I claim:

1. A method of producing a unified monolithic building product in sheet form which comprises forming a

gelatinous cellulosic binder by dispersing a kraft fiber in water to form a slurry of up to about 6% consistency, continuously passing the slurry through a series of pulp refiners having abrading surfaces preset to gelatinizing conditions for a time and an intensity to produce an essentially nonfibrous gelatinous slurry having a Schopper-Riegler freeness of up to about 100 ml., and a particle size on the order of up to about 0.06 mm., admixing the resulting slurry with from 5/3 to 9 parts of a thermally expanded perlite per part of binder (dry basis) to form an aqueous slurry of a consistency of from 4 to 8 percent, the major proportion of said perlite having a particle size of greater than 200 mesh, forming a felted sheet from said admixture, compressing the felted sheet to expel excess water, and drying said sheet.

2. The process of claim 1 wherein the proportion of thermally expanded perlite admixed with cellulosic binder is from about 7/3 to 8.5 parts of perlite per part of cellulosic binder (dry basis).

3. The process of claim 1 wherein a wax emulsion in an amount of up to about 2 percent by weight (dry basis) is added to said aqueous admixture.

4. The process of claim 1 wherein the abrading surfaces are lava.

5. A lightweight unified monolithic building product in sheet form, said unified product comprising a mechanically induced water activated cellulosic gelatinous binder having a Schopper-Riegler freeness in its original hydrated state of less than about 100 ml. and prepared from a slurry of kraft paper fibers of a consistency of up to about 6 percent which is subsequently gelatinized by passage through a series of paper refiners preset to gelatinizing conditions to produce a cellulosic binder having an average particle size on the order of up to about 0.06 mm., and from 5/3 to 9 parts of a thermally expanded perlite, the major proportion of which has a particle size of greater than 200 mesh, said unified product being further characterized in that the unification is provided by the essentially nonfibrous substance acting essentially as an adhesive without fiber interfelting action.

6. The product of claim 5 containing a minor proportion, with respect to the amount of perlite, of ceramic clay.

7. The product according to claim 5 wherein the thermally expanded perlite is present in proportions of from about 7/3 to 8.5 parts per part of cellulosic binder (dry basis).

8. The product of claim 5 wherein a paper sheet is laminated on at least one surface of said dried sheet.

#### References Cited

##### UNITED STATES PATENTS

|              |         |                |           |           |
|--------------|---------|----------------|-----------|-----------|
| 2,426,923    | 9/1947  | Cowles         | -----     | 162—187   |
| 2,634,207    | 4/1953  | Miscall        | -----     | 162—181   |
| 55 2,971,878 | 2/1961  | Heilman et al. | 162—181 X |           |
| 3,001,907    | 9/1961  | Bergstrom      | -----     | 162—181 X |
| 3,066,065    | 11/1962 | Koerner et al. | -----     | 162—187 X |

DONALL H. SYLVESTER, Primary Examiner.

60 HOWARD R. CAINE, Examiner.